

3,153,825  
**CARBON-BONDED REFRACTORY CASTING MOLD  
AND PROCESS FOR FABRICATION THEREOF**  
Bryant W. Crocker, Reading, Mass., assignor to the United  
States of America as represented by the Secretary of  
the Army  
No Drawing. Filed Jan. 8, 1962, Ser. No. 165,045  
4 Claims. (Cl. 22—193)  
(Granted under Title 35, U.S. Code (1952), sec. 266)

The invention described herein may be manufactured and used by or for the Government for governmental purposes without the payment to me of any royalty thereon.

This invention relates to the forming of the molds and cores employed in foundry casting operations and is directed more particularly to a method of treating resin-bonded refractory sands, as well as metal powders, to provide relatively fine-grained molds of superior strength and surface finish which will not react with the molten metal being cast therein.

Considerable difficulty has been encountered in the development of suitable molds and cores of the type utilized in the precision casting of refractory metals such as titanium and uranium which possess an unusual affinity for oxygen. While the major source of oxygen contamination can be eliminated through the expedient of melting and pouring the metal to be cast in a vacuum, the successful precision casting of chemically active refractory metals is still faced with the problem of developing an inert mold which can be easily and economically fabricated. Extensive research in this area has shown that the minimum contamination in the metal being cast is achieved through the use of various forms of carbonaceous material. Consequently, current practice in the fabrication of precision casting molds and cores is to machine them from solid blocks of graphite. However, this procedure is not only extremely costly but produces molds of poor permeability and tends to promote the formation of cold shuts or laps during the solidification of the metal being cast. While some of these undesirable characteristics can be avoided through the utilization of graphite which is rammed into the mold configuration and thereafter sintered, the processing of this type of material is not only expensive but is subject to the problem of dimensional sensitivity.

It has been found that the use of relatively thin-walled disposable molds composed of a refractory sand or powder held together by a thermosetting plastic or resin is particularly well suited to the production of precision castings. However, these molds, which are generally referred to as "shell molds," are not presently employed in vacuum casting in view of the large volume of gases and other volatiles which are evolved during the burning to which the resin binder is subjected upon contact with the molten metal being cast. The proper escape of these gases requires a mold material of relatively high permeability which, of course, involves a corresponding reduction in the attainable strength thereof.

Accordingly, it is a principal object of this invention to provide a relatively simple and inexpensive process of forming the molds and cores utilized in precision casting techniques such that the finished product may be successfully employed in vacuum casting without imparting any significant contamination to the metal being cast therein.

A further object of this invention is to provide a more economical method of forming thin-walled shell molds capable of imparting a better surface finish and dimensional stability to vacuum castings than has been heretofore possible with molds of graphite construction.

Still another object of the present invention is the provision of a process wherein either a refractory sand or metal powder is bonded by a thermosetting resin and treated in a vacuum to eliminate any subsequent release of combustion gases during contact with the metal being cast.

A particular object of this invention lies in the provision of a method for converting the resin bond of a shell-type refractory sand mold to a carbon bond of considerably greater strength without any significant change in dimensions.

It has been discovered that the foregoing objects may be achieved by subjecting a shell mold of zircon bonded with phenol-formaldehyde to a temperature of about 1650° F. within a vacuum of about 20 microns for a period of time sufficient to drive off all gases and other volatiles evolved during the conversion of the resin to carbon. Such treatment results in an unexpected improvement in the molds and cores which are utilized in the precision casting of such refractory metals as titanium and uranium since it provides a strong, smooth material of variable permeability which will not significantly contaminate the metal being cast thereagainst.

Present-day shell molding techniques generally utilize silica in the form of sand as the refractory material from which the mold is fabricated. However, inasmuch as silica will react with carbon and form silicon and carbon dioxides at the temperatures and vacua required to completely carbonize the resin, the present invention utilizes zircon as the preferred refractory for the mold material. However, experimentation has shown that other refractory silicates, oxides, as well as metal powders, may be employed as a satisfactory substitute for the zircon. For example, it has been found that copper is one of the metals which will not seriously contaminate the type of refractory metal to be cast and, consequently, when employed in suitable powder form will produce results which are at least equivalent to those obtained with zircon sand. The size of the individual grains of the refractory material or metal powder is, of course, dependent upon the degree of surface finish desired in the solidified castings. If an extremely fine finish is required, the grain size of the zircon should be reduced to provide a "flour" rather than the "sand" type in normal usage.

While any thermal or air-setting organic plastic may be employed to bind the refractory material, it has been found that the phenol-formaldehyde resin generally utilized in shell molding is preferred for reasons of economy. However, extremely successful results have been achieved with a furan air-setting resin and a catalyst which enables the resin to polymerize at room temperature. The resin may be either wet or dry but in the event it is utilized in the latter form, it is essential that the ingredients be thoroughly mixed to provide substantially uniform distribution.

Although the percentages by weight of the resin and zircon will vary in accordance with the particular characteristics desired in the mold, maximum strength and hardness has been achieved with a mixture of 88% zircon flour and 12% resin. A mixture of 45% zircon flour, 45% zircon sand of AFS No. 130 fineness, and 10% resin has also given excellent results. If greater mold permeability is desired, this may be accomplished with a mixture of 93% zircon sand of AFS No. 130 fineness and 7% resin. The important characteristics obtained with these mixtures are listed below in Table I and are compared with the corresponding results achieved with a standard shell mold and an oil core mold.

3  
Table I

| Mix             | Scratch Hardness | Dry Permeability Number | Fiber Stress (p.s.i.) | Mold Shrinkage (in./in.) | Mold Hardness |
|-----------------|------------------|-------------------------|-----------------------|--------------------------|---------------|
| 88-12           | 94               | 12                      | 1,938                 | .026                     | 100           |
| 45-45-10        | 87               | 12                      | 1,500                 | .010                     | 100           |
| 93-7            | 55               | 60                      | 200                   | .006                     | 100           |
| Std. Shell Mold | 98               | 60                      | 850-1,100             | .002<br>(max.)           | 100           |
| Oil Core Mold   | 70-90            | 40-140                  | 150-200               |                          | 90-100        |

As shown in this table, the fiber stress or transverse strength of the molds fabricated from the mixture of 88% zircon sand and 12% resin is virtually double that provided by the shell molds treated in a conventional manner.

Once the selected mixture has been milled to the desired extent, the shell molds may be formed to shape and cured in the conventional foundry manner. However, instead of subjecting the molds to the customary baking procedure, they are placed in a vacuum furnace whose controls are set to provide a vacuum of about 20 microns. While 10 to 30 microns constitutes a preferred range, satisfactory results can be achieved with vacuum systems ranging as high as 1000 microns. Thereafter, the furnace temperature is raised to about 1650° F. Experimentation has shown that temperatures below 1400° F. will not provide the desired complete carbonization of the resin while temperatures above 2000° F. will result in an undesirable chemical reaction between the zircon and the carbon which is formed by the decomposition of the resin. The desired furnace temperature is maintained until operation of the vacuum pump signals that the carbonization of the resin has been completed and that no further combustion gases will be evolved. The duration of this heating step is, of course, dependent upon the size and section thickness of the mold. Thereupon, the furnace temperature is lowered to about 400° F. to permit the molds to cool sufficiently for subsequent removal from the furnace. At this point, the molds can be prepared in the usual manner to receive the molten metal to be cast therein.

In view of the absence of atmospheric pressure on the mixture of zircon and resin, the rapid evolution of the hydrocarbons and other volatiles produced by the burning of the resin is accompanied by an unusual frothing and foaming action which thoroughly distributes the carbon residue among the individual grains of the zircon sand. Although it is not definitely known whether the carbon and zircon undergo a chemical reaction or a physical diffusion, it is apparent that the intimate contact between the carbon and zircon results in actual bonding at the interface surfaces thereof. The temporary binding action of the resin is thus converted to an interconnected skeletonized carbon structure which surrounds and holds the zircon grains so as to form an unusually strong and rigid mold. Inasmuch as the carbonizing temperature is first attained at the outer surface of the mold and then gradually pervades the inner regions thereof, the aforementioned foaming action of the resin binder occurs on a progressive local basis which does not alter the external dimensions of the mold to any measurable extent.

Chemical analysis of various molds produced in accordance with this invention has shown that the resin is almost entirely reduced to amorphous carbon with the retention of only 0.085 percent by weight of hydrogen. As a result, either titanium or uranium may be cast into these molds with no significant surface contamination. Furthermore, unlike conventional shell molds, the structural rigidity of the mold itself will not be seriously weakened by the high temperatures of the molten metal being poured therein. Moreover, the absence of gas formation during the pouring of the casting permits an appreciable reduction in the permeability required for the

5 mold material thereby enabling the use of a much finer particle size for the zircon which provides a much finer surface finish as well as greater strength and rigidity. It has been found that molds prepared in accordance with this invention may also be used for the casting of bronze, copper, aluminum, magnesium, and various steel alloys with excellent results.

10 It can, therefore, be seen that a resin-bonded mold of refractory sand or even a metal powder treated in a vacuum furnace in the manner described above will provide sound precision castings in a variety of metals over a wide range of casting temperatures.

15 Although a particular embodiment of the invention has been described in detail herein, it is evident that many variations may be devised within the spirit and scope thereof and the following claims are intended to include such variations.

I claim:

1. A process for treating shell molds formed of a mixture of zircon sand and a thermosetting resin polymerized into a temporary binder for the sand comprising the steps of completely carbonizing the resin at a temperature of about 1650° F. within a vacuum of about 20 microns, continuously exhausting the combustion gases produced by the burning of the resin, and thereafter cooling the heated molds to a temperature of 400° F. prior to removal from the vacuum.

2. A method of increasing the transverse strength of a shell mold formed of a mixture, by weight, of 88% zircon sand and 12% phenol-formaldehyde resin which comprises the steps of completely converting the resin to an essentially 100% pure amorphous carbon by subjecting the molds to a temperature of about 1650° F. within a vacuum of less than 20 microns, continuing the heating until the evolution of the combustion gases is completed, and thereafter cooling the heated molds to a temperature of about 400° F. prior to the removal thereof from the vacuum.

3. A casting mold characterized by relatively low permeability, high transverse strength, and a virtual absence of contaminating effect on molten refractory metals such as titanium and uranium, said mold consisting essentially of a major proportion of zircon sand and a minor proportion of amorphous carbon surrounding the individual grains of zircon sand uniformly throughout the mold, said carbon being the result of the complete conversion, within a vacuum, of the polymerized resin utilized to temporarily bond the zircon sand into mold form.

4. A method of bonding a metal powder with substantially pure carbon to provide a mold into which molten metal may be cast without contamination, comprising the steps of coating the individual particles of powder with a phenol-formaldehyde resin, polymerizing the resin to temporarily bind the powder into the desired shape of the mold, heating the mold to a temperature of about 1650° F. in a vacuum of 10 microns for a sufficient period of time to completely convert the resin to substantially pure carbon, and cooling the heated mold to about 400° F. prior to removal from the vacuum to permanently bond the metal powder into a material which will be relatively chemically inert when in contact with the molten metal being cast.

References Cited in the file of this patent

UNITED STATES PATENTS

- 2,548,897 Kroll \_\_\_\_\_ Apr. 17, 1951  
2,772,457 Webbers \_\_\_\_\_ Dec. 4, 1956  
3,023,119 Anderson et al. \_\_\_\_\_ Feb. 27, 1962

FOREIGN PATENTS

- 187,247 Australia \_\_\_\_\_ Oct. 25, 1956  
834,864 Great Britain \_\_\_\_\_ May 11, 1960

OTHER REFERENCES

The Iron Age, November 23, 1961, pages 76 and 77.